

## UNITED STATES PATENT OFFICE

2,032,992

## WOVEN OR KNITTED FABRIC MAINLY CONSISTING OF CELLULOSIC FIBERS AND METHOD OF MANUFACTURING SAME

Richard Lant, Vienna, Austria

No Drawing. Application August 24, 1933, Serial No. 686,654. In Austria September 6, 1932

5 Claims. (Cl. 8—20)

According to British Patent No. 343,104 it has been proposed to treat or esterify woven or knitted fabrics with higher fatty acid chlorides in presence of pyridine.

Now it has been observed that if woven or knit fabrics mainly consisting of cellulose containing fibers are provided on at least one side with a uniform dense downy coating consisting of cellulose fibers projecting from the fabric and produced for instance by teasing, carding or grinding and by subsequent shearing, if so desired, for more or less shortening the fibers, and if then the fabric is esterified in a manner substantially known per se with higher fatty acids, a product is obtained which shows a surprising deer skin like touch on the side or sides provided with the said downy coating. It has already been attempted to impart to textile fabrics a leather like touch by various other methods such for instance as grinding but this can be arrived at only to a very slight extent. On the other hand by esterifying a fabric not ground or teazled no leather like touch can be obtained. Therefore it is highly surprising that to a fabric mechanically prepared by grinding and, if desired, subsequent shearing a highly leather like touch heretofore unknown may be imparted by the aforesaid esterification, the touch being that of a firm leather if the downy coating produced by teasing, carding or grinding has been cut down to a great extent by shearing, whereas without such shearing the touch is that of a softer leather.

Fabrics prepared as above described are very suitable for the manufacture of various articles such as gloves, bags, hats and the like.

The following is an example of a preferred operation of the process according to this invention.

Knitted cotton fabric such as glover's cloth, is provided with a layer (down or fuzz) of single fibers projecting from the cloth. This is done for instance by raising or carding and eventually warping the fabric on at least one side. Alternatively already "roughened" knitted cotton fabric can be used as available on the market. In either case 4 kg. stearine acid chloride dissolved in 40 kg. of pure pyridine are caused to act upon 10 kg. of such fabric which is provided with a layer of single fibers on at least one side as above described, the fabric being practically absolutely dry. The reaction is effected in a closed receptacle so that air and moisture are excluded, at a temperature of 95 to 100° C. for about half an hour. By carefully moving the fabric to and fro in the reagent, as much as is possible of an even and thorough impregnation of the cotton knitting

with the solution of the stearine acid chloride is effected. After termination of the reaction the fabric is carefully neutralized, cleaned if necessary with the aid of chemical means and thoroughly washed.

When treated according to the above mentioned conditions of reaction the fabric acquires an additional weight caused by the esterification amounting to from 20 to 25% of the original weight of the dry fabric. By changing the time or the temperature of reaction and especially by changing the quantity of acid chloride the extent of the esterification can be changed, i. e. the increase of weight of the fabric obtained by esterification. For the purposes of this invention various degrees of esterification are suitable, which may be defined by the amount of increase of weight of the dry fabric to be treated, which lies within the range of from 5% to 30%. Below this stated lower limit of esterification the desired feel of the firstly fluffy side or sides, resembling more or less smooth buckskin is not obtained to the extent which is desirable for practical purposes. The feel improves gradually with the increase in the degree of esterification, e. g. 8% giving a better feel than 5%. An esterification surpassing the higher limit above indicated will not further improve the feel and may possibly impair the strength of the fabric.

The most advantageous limits of esterification can be defined by an increase in weight of the dry starting material of 15 to 25%. If it is desired to obtain finally a product of white colour, then the cloth obtained as above described can be bleached, while if coloured products are to be obtained, the fabric can be dyed before the esterification with substantive dyestuffs. If it seems advisable in view of some reason or the other, the order of treating can be changed, but if it is intended to dye after the esterification has taken place, then other dyestuffs must be used e. g. those which are suitable for dyeing artificial acetate silk.

Woven or knitted fabrics are preferred as starting material as above described. In some cases eventually also other manufactured coherent structures formed from or containing mainly cellulosic material can be used, such for example as coherent felted structures.

The esterification can be effected in any suitable apparatus such for example as that as described in the British Patent No. 376,295.

The combination of two steps are essential for the effect to be achieved: Providing firstly a fuzz (down) on at least one side of a woven or knit-

ted fabric consisting of or containing in the main part cellulosic fibers and secondly esterification of the fabric with higher fatty acids in a manner known per se. This process results in a new improved industrial product, namely a web or knitting consisting essentially of cellulosic fibers and having on at least one side a layer of smooth buckskin-like feel, the layer forming a single piece with the fabric.

10. The invention here described and claimed includes the process and the improved fabric thereby obtained.

Articles manufactured from this material as e. g. gloves, bags, hats and the like are also included in this invention and claimed herewith.

15. What I claim is:

1. The process which consists in providing a woven or knitted fabric containing essentially cellulosic fibers on at least one side with a down 20 of cellulosic fibers projecting from the fabric and causing higher fatty acid chlorides dissolved in pyridine to act upon the dry fabric together with the down of cellulosic fibers until an increase in weight caused by esterification of 5 to 30% of the 25 dry fabric is obtained.

2. The process which consists in providing a woven or knitted fabric containing essentially cellulosic fibers on at least one side with a down of cellulosic fibers projecting from the fabric and causing stearine acid chloride dissolved in pyridine to act upon the dry fabric together with the 30

down of cellulosic fibers until an increase in weight caused by esterification of 5 to 30% of the dry fabric is obtained.

3. The process which consists in providing a woven or knitted fabric containing essentially 5 cellulosic fibers on at least one side with a down of cellulosic fibers projecting from the fabric and causing stearine acid chloride dissolved in pyridine to act upon the dry fabric together with the down of cellulosic fibers until an increase in 10 weight caused by esterification of 15 to 25% of the dry fabric is obtained.

4. As a new article of manufacture a woven or knitted fabric containing essentially cellulosic fibers and having on at least one side a down of 15 cellulosic fibers projecting from the fabric, said cellulosic fibers of the fabric and down being partially esterified with higher fatty acids from 5 to 30% by weight of the original fabric, the fabric having a smooth feel resembling the feel 20 of buckskin and being water repellent.

5. As a new article of manufacture a woven or knitted fabric containing essentially cellulosic fibers and having on at least one side a down of 25 cellulosic fibers projecting from the fabric, said cellulosic fibers of the fabric and down being partially esterified with higher fatty acids from 15 to 25% by weight of the original fabric, the fabric having a smooth feel resembling the feel 30 of buckskin and being water repellent.

RICHARD LANT.